

## UNITED STATES PATENT OFFICE

FRANK R. PALMER, OF READING, PENNSYLVANIA, ASSIGNOR TO THE CARPENTER STEEL COMPANY, OF READING, PENNSYLVANIA, A CORPORATION OF NEW JERSEY

## ANTIFRICTION CORROSION-RESISTING STEEL

No Drawing.

Application filed January 17, 1928. Serial No. 247,462.

My invention has for its object the production of alloy steels of the corrosion or scale resisting class, which will be characterized by what may be best termed anti-friction properties as evidenced by their behavior when in kinetic contact with tool material employed in their fabrication or with surface material in connection with which they are used.

10 In the corrosion and scale resisting or "stainless" steels to which my invention particularly relates; the element chromium is used in high percentages relative to the iron or steel base, with or without other alloying elements such as nickel, copper, molybdenum, silicon or tungsten; the minimum chromium content for scale resisting quality being about 2.00%, and for corrosion resisting quality about 8.00%. It has been found however 20 that all of these high-chromium steels incidentally possess a characteristic quality which is not only unsought for but which is generally objectionable; namely, what may be termed a gummy or sticky quality 25 which causes such steels to adhere to other materials with which they are brought into kinetic contact. This high-friction quality of these corrosion resisting steels impairs their machinability independently of recognized anti-machining qualities such as inherent hardness or a tendency to work-harden; the high-friction quality referred to causing sticking of chips to tools or of fragments 30 of the metal to abrasive mediums, with resulting difficulties and imperfections; and also impairing the usefulness of properly finished articles made therefrom so far as kinetic friction is involved, by tending to cause cutting or galling and even freezing or seizing of the 35 contacting surfaces.

It is generally known that this high-friction quality of these high-chromium corrosion resisting steels is much greater than it 45 is in ordinary straight carbon steels, and that it is not due to differences in surface hardness or physical properties as ordinarily determined, but seems to be inherent in the analysis of these high chromium alloy steels. 50 The high-friction characteristics of such

steels are evidenced clearly by the following examples:

In order to satisfactorily cold-draw wire, tubing, etc., from usual high-chromium steels it is necessary that they be plated with 55 a non-ferrous metal so as to avoid actual contact with the drawing die—otherwise the metal will adhere to the die. Bolts and nuts may even become frozen upon screwing them together by hand. In machining, chips are 60 apt to adhere so firmly to the tool as to seriously interfere with the work. In moving parts operating at elevated temperatures such as for instance high pressure gate valves and poppet valves, made of this otherwise desirable material, this high-friction quality tends to cause galling, sticking or freezing. The field of satisfactory usefulness of high-chromium corrosion resisting steels is thus 65 materially reduced.

The above examples are typical of a real problem involved in the commercial use of high chromium corrosion and scale resisting steels for which there has hitherto been no adequate solution. The purpose of my invention is to overcome these disadvantages, 70 which have been long accepted as inherent in these steels, and to attain this purpose without sacrifice of desired qualities; the invention consisting in the production of a new 75 alloy steel as hereinafter fully described, in which the desired corrosion resisting qualities are retained and this deleterious high-friction quality is substantially neutralized.

In all stainless and other high-grade steels, 80 the metalloid sulphur appears incidentally, but is hardly tolerated in quantities exceeding about .05%; though in the common straight carbon product known as screw stock, the sulphur may be permitted as high 85 as .15% to improve machinability. I have found that sulphur, when incorporated in relatively large amounts in a high chromium corrosion of scale resisting steel, will offset 90 the high-friction qualities which are present 95 by reason of the high chromium. It was found in the development of this invention that percentages of sulphur—even as high as that used in common screw stock—had little 100 effect on either the machinability or fric-

tional characteristics of high-chromium corrosion resisting steels. When quantities of sulphur in excess of about .15% were introduced into a corrosion resisting steel base, it was found that the hot working qualities 5 were so decreased as to make the satisfactory forging or rolling of the resultant steels very difficult; but in spite of this fact I have melted these corrosion resisting alloys with sulphur contents ranging from .15% up to 10 .180%, and these were tested in the condition as cast. For corrosion resisting steels containing more than 10.00% chromium, it was found that the desired anti-friction properties sought for were realized with a sulphur 15 content of .30% or more. Between .15% and .30% sulphur the improvement is progressive, the results becoming entirely satisfactory at about .30% sulphur, and not being proportionately improved by larger quantities 20 of sulphur. When the chromium content falls below 10% into the range principally used for scale resisting purposes, the percentage of sulphur required for anti-friction qualities may be reduced to as low as 25 .10%.

My improved alloy as described above may be satisfactorily employed for castings with desired anti-friction effect but for malleable 30 steels objectionable red-shortness caused by resulting iron-sulphide is apt to result. In experimenting in a crucible furnace with a view to overcoming this bad effect of the relatively large content of sulphur required to 35 offset the high-friction quality of high chromium steels, primarily dealt with, I have found that this can be quite satisfactorily accomplished by proper addition of zirconium, an element known to decrease red-shortness due to high sulphur, and a small quantity of 40 which I have ascertained may be effectively and satisfactorily employed in these high-chromium corrosion resisting steels, in connection with the high sulphur content which I have employed to neutralize their high-friction quality; with the desired result of 45 correcting the red-shortness otherwise produced, and without impairing the desired effect of the sulphur or without deleterious effect upon the desired qualities imparted by 50 the high-chromium of such steels. I have found, in the crucible furnace product made, that the addition of about .25% of zirconium to the molten bath fully corrects the red-shortness produced by a sulphur content of 55 .30%, the residual content of zirconium in the steel after loss in the molten bath being about .12% which combines with the sulphur as commonly understood to form a finely divided slag like inclusion. The required zirconium is readily introduced by using silicon-zirconium without detrimental silicon effect the silicon in fact serving to supplement 60 the chromium used.

65 The percentage of zirconium employed va-

ries with the sulphur content and a moderate excess of zirconium produces no harmful effect. Satisfactory results may be secured by keeping the residual zirconium content about one-half the sulphur content of the steel. 70

It should also be understood that the red-short effect of the high sulphur may be offset by the use of abnormally high manganese additions to the metal, or by manganese and zirconium jointly, but because of the collateral effects of high manganese, I prefer to use zirconium in most instances. 75

A typical example of my improved alloy steel has been variously used as hereinafter set forth, so as to clearly demonstrate how effectively my invention has neutralized the high-friction characteristic of high-chromium corrosion resisting steels, with full retention of desired corrosion-resisting qualities; the analysis of this example so far as main 80 elements are concerned, being as follows:

|           | Per cent |
|-----------|----------|
| Carbon    | .10      |
| Chromium  | 14.00    |
| Sulphur   | .30      |
| Zirconium | .12      |

Hot rolled wire rods made from steel of this analysis, have been cold drawn without any metallic coating—in the same manner as straight carbon steel and with equal avoidance of seizing, galling or scratching. Steel of the same analysis has been subjected to turning, milling, drilling, tapping and threading operations by ordinary steel-cutting tools, with the same facility and smoothness of finish as straight-carbon steel, the cutting edges of the tools remaining equally free of adhering "bugs". Similar cylindrical weights made respectively from steel of the above analysis and from like high-chromium steel with minimum sulphur and zirconium elements, when placed on a polished inclined plane have shown markedly quicker starting and sliding movement by the former. When subjected to salt-water spray testing conditions, my improved alloy steel shows the same corrosion-resisting quality as does like high-chromium steel which is minus the sulphur-zirconium addition. 110 115

The above analysis is not to restrict in any way the scope of my invention as I have similarly added sulphur and zirconium to corrosion resisting steels of both higher and lower chromium contents both with and without the addition of other elements such as silicon, copper and nickel, and the improvement was of the same order, it being readily understood that the desired anti-frictional effect is conferred by the considerate providing of an abnormally high sulphur content, and further that these high-chromium, high-sulphur steels are made more malleable by the coating zirconium element as described. 120 125 130

in an electric furnace as usual, the sulphur and zirconium being readily added to the base alloy steel as determined by good steel making practice; it being readily understood  
5 that an excess amount of sulphur and zirconium must be used in order to secure a desired yield, and my present experience showing apparent advantages in dumping a portion of lump sulphur with a smothering  
10 layer of silicon-zirconium or ferro-zirconium, upon the bottom of the ladle as the heat is tapped, and throwing a further supply of sulphur into the flowing stream, this method yielding about fifty per cent of the quantity  
15 of sulphur and zirconium used.

What I claim is:

1. As a composition of matter, a corrosion-resistant alloy steel containing essentially between 7% and 30% of chromium, and between .15% and 1.80% of sulphur, and characterized by an anti-friction quality.
2. As a composition of matter, a corrosion-resistant alloy steel containing essentially between 7% and 30% of chromium, between .15% and 1.80% of sulphur, and between .05 and 2.00% of zirconium, and characterized by anti-friction quality.
3. As a composition of matter, a corrosion-resistant alloy steel containing essentially between 10% and 20% of chromium, and between .15% and 1.00% of sulphur, and characterized by anti-friction quality.
4. As a composition of matter, a corrosion-resistant alloy steel containing approximately 14% of chromium, and .30% of sulphur, and characterized by anti-friction quality.
5. As a composition of matter, a corrosion-resistant alloy steel containing essentially between 8% and 20% of chromium, and between .15% and .25% of sulphur, and characterized by anti-friction quality.

In testimony whereof I affix my signature.

FRANK R. PALMER.

45

50

55

60